

Jan. 30, 1968

J. E. BROWN ET AL

3,365,768

METHOD FOR MAKING STRETCH YARNS AND FABRICS

Filed April 28, 1964

3 Sheets-Sheet 1



FIG. 1

Inventors  
James E. Brown  
William Frank Taylor  
By their attorneys

Hanson and Hanson.

Jan. 30, 1968

J. E. BROWN ET AL

3,365,768

METHOD FOR MAKING STRETCH YARNS AND FABRICS

Filed April 28, 1964

3 Sheets-Sheet 2



FIG. 2

Inventors  
James E. Brown  
William Frank Taylor  
By their attorneys  
Hauson and Hauson.

Jan. 30, 1968

J. E. BROWN ET AL

3,365,768

METHOD FOR MAKING STRETCH YARNS AND FABRICS

Filed April 28, 1964

3 Sheets-Sheet 3



FIG. 3

FIG. 4

FIG. 5



Inventors  
James E. Brown  
William Frank Taylor  
By their attorneys

## 1

3,365,768

METHOD FOR MAKING STRETCH  
YARNS AND FABRICS

James E. Brown, Axis, and William Frank Taylor, Mobile, Ala., assignors to Courtaulds North America Inc., New York, N.Y., a corporation of Alabama

Filed Apr. 28, 1964, Ser. No. 363,250

11 Claims. (Cl. 28—76)

This invention relates to stretch yarns and fabrics and to a method for their production.

It is known to make stretchy yarns and threads from cellulosic materials by impregnating them with elastomeric materials such as rubber. However, such yarns are obviously limited in the uses to which they may be put. Moreover, it is found that most stretch yarns are difficult to handle on conventional textile machinery simply because of their stretchiness.

The present invention provides a way to make stretch yarns which are predominantly cellulosic and which are therefore relatively inexpensive. Yarns according to the invention have the advantage of temporarily losing their stretch when wound on spools so that they can be woven or knitted as conventional, non-stretch yarns on ordinary textile machinery. The stretch can then be fully redeveloped merely by wetting the fabric.

In accordance with the invention, a stretch yarn is made by treating a plied yarn, comprising cellulose filaments and from about 3% to about 25% by weight thermoplastic filaments, in the absence of tension, with a cellulose swelling agent equivalent to an aqueous solution containing 5 to 40% NaOH, and heating the yarn to a temperature sufficient to plasticize the thermoplastic filaments.

Following heating the yarn may be back twisted, if desired.

Yarns made in accordance with the process just described, prior to back twisting, have the form of a close helix. The thermoplastic filaments have the shape required by the helix and have acquired a memory for that shape through heat setting. Upon back twisting, a three-dimensional irregular yarn is produced having a sequence of sections comprising closely wound helices and uncoiled sections in which the individual plies are separated from one another and sprung outwardly from the main axis of the yarn.

In making stretch fabrics according to the invention, yarns made as described above may be pulled out and retained in an extended position until they fail to return to the contracted form upon release. No special technique is required for this, since if the yarns are spooled under tension sufficient to pull the yarn out, by the time the spools have been transferred to a loom or knitting machine, the recovery will have been lost. The fabric may then be manufactured by any conventional technique, using the yarn as though it had never had stretch properties. After the fabric is made, it may be washed or steamed to redevelop the stretch properties.

Alternatively, fabric may be made from a plied yarn containing 3 to 25% thermoplastic filaments and the balance cellulose filaments, and then treated slack with a swelling agent of the class described, followed by heat setting of the thermoplastic filaments. In general, however, it is more desirable to treat the yarn as yarn, prior to making it into fabric.

In the drawings:

FIG. 1 is a flow diagram illustrating the process for making stretch yarn according to the invention.

FIG. 2 is a flow diagram illustrating the preferred process for making stretch fabric in accordance with the invention.

## 2

FIG. 3 is a flow diagram illustrating another method for making stretch fabric according to the invention.

FIG. 4 shows a stretch yarn made in accordance with the invention without reverse twisting.

FIG. 5 shows the yarn of FIG. 4 after reverse twisting.

Referring first to FIG. 1, the first stage in making stretch yarns according to the invention is to obtain a plied yarn containing 3 to 25% thermoplastic filaments and the balance cellulose filaments.

The thermoplastic filaments useful in the present invention may be any of those available on the market. They need only be capable of softening or plasticization by heat, at temperatures which will not adversely affect cellulose, say at less than 200° C. Among the substances that may be used as the thermoplastic component there may be mentioned cellulose esters, polyesters such as polyethylene terephthalate, acrylic polymers, for example polyacrylonitrile and polyolefins such as polyethylene or polypropylene.

The cellulose filaments may be natural cellulose fibers such as cotton, ramie, jute or linen, or regenerated cellulose fibers whether made by the viscose, cuprammonium, nitrate, or other conventional processes such as the saponification of cellulose acetate. Preferably, however, if regenerated cellulose fibers are used, they will be the so-called "polynosique" or high wet modulus fibers. This is a comparatively recent type of viscose rayon fiber characterized by a generally circular cross-section (in a direction perpendicular to its axis), a substantially smooth, non-crenulated skin, with no apparent skin-core structure, and a fine microfibrillar structure. As a class polynosique fibers are characterized by a much higher resistance to swelling in water or caustic soda than is conventional viscose rayon. They are often referred to as

"high wet modulus" fibers because the wet modulus, i.e., the stress required to cause an elongation of a specified amount when the fiber is wet, is much greater than is the case with conventional rayon, amounting to greater than 1 gram per denier stress for a 5% elongation.

Fibers of this type may be made by extruding unripened viscose into a coagulating bath weak in regenerative power and stretching the filaments to a very high degree prior to or simultaneously with regeneration. See Tachikawa 2,732,279 and Cox 2,937,070.

Conventional rayon is preferably not used as the cellulose component in the yarns of the invention in proportions greater than 90% of the weight of the yarn. The reason for this is that with treating solutions of the type described, conventional rayon tends to become gelatinized, so that when proportions of more than 90% are present the final product tends to be stiff, brittle and inflexible.

The thermoplastic and cellulose filaments may be assembled in various ways. In the preferred embodiment the singles yarns are made up of a blend of cellulose staple and thermoplastic staple and these single yarns are then plied. Alternatively, continuous individual thermoplastic filaments may be twisted with individual continuous filaments of rayon to make up the singles yarn.

Again, in plying the yarn, a yarn of thermoplastic filaments, which may be continuous or staple, may be plied with a yarn or yarns of cellulose fibers, either continuous or staple. Regardless of how the components are selected or assembled, the weight proportion of thermoplastic filaments in the plied yarn should be between about 3% and about 25% based on the weight of the combined yarn.

The individual singles yarns which are plied preferably have from about 10 to about 40 twists per inch. The plied yarn itself must have at least two plies and may have up to say 6 plies. The plied yarn is preferably twisted to the opposite hand from the singles yarns, and the singles

yarns are preferably all twisted to the same hand. The plied yarn will have from say 5 to 40 twists per inch.

As will be seen from FIG. 1, the first step in the novel process is subjecting the plied yarn to a swelling treatment. The preferred swelling agent is caustic soda of 5 to say 40% concentration. The precise concentration employed will vary with the cellulosic fiber being treated, since even among cellulose fibers of the same general class, there is some variation in the effect of different caustic concentration. In place of caustic soda, other alkali metal hydroxides, e.g., KOH, may be used, as well as such materials as zinc chloride and sodium zincate. Where swelling agents other than sodium hydroxide are used their concentrations are selected to give a swelling effect equivalent to that of sodium hydroxide in concentrations of 5 to 40%.

The swelling treatment is preferably carried out at room temperature (20° C.), but other temperatures ranging from 0° C. to 80° C. may be employed if desired. In accordance with well known principles lower temperatures enhance the swelling effect.

The time of treatment depends on many factors, including the concentration of swelling agent, the temperature, the physical size of the yarn and mechanical details of the impregnating apparatus. In general the contact time of the yarn and swelling solution will range from say .1 to 120 minutes.

The swelling treatment is carried out in the substantial absence of tension. This may be done by passing the yarn, hanging in a catenary, through a bath of the swelling agent, laying the yarn in plaited form on a conveyor passing through a bath or under a spray, suspending skeins of the yarn in a bath, or in any other convenient way. In any event, the yarn must be free to contract, for in this swelling treatment the yarn assumes the form shown in FIG. 4. As shown in that figure, the yarn coils upon itself to form a tightly wound helix, the succeeding coils of which are substantially contiguous and the helix angle approaches 90° (say 45° or more).

Following the swelling treatment, the yarn may be neutralized, for example with a dilute solution of acetic acid, washed and dried.

In accordance with the invention, the yarn is next heated to a temperature sufficient to plasticize or soften the thermoplastic filaments. This temperature must not be so high as to melt the thermoplastic but it must be sufficiently high so that, after cooling, the thermoplastic filaments develop a memory for the form they assumed by virtue of the coiling of the yarn, and will therefore tend to return to that configuration. This temperature will, of course, vary with the particular thermoplastic filament being used. Generally it will be between about 120 and about 200° C. The heating is also carried out with the yarn slack, i.e., in the substantial absence of tension. Conveniently it may be done by passing the yarn in air through a conventional drier or oven in a loop or catenary.

The yarn which is obtained as a product after the heat setting treatment will have the bulky, coiled form described above.

The yarn in the close helix form may now be wound on spools and used to make fabric, as outlined below. Preferably, however, the yarn is reverse twisted, i.e., it is twisted to a direction opposite to that in which it was plied. The degree of reverse twist may range from say 80 to 200%, preferably from 135 to 160% of the twist applied during plying.

The effect of the reverse twist is shown in FIG. 5. As may be seen from that figure, the yarn is an irregular three dimensional sequence of helical sections, the helix angle of succeeding sections varying in an arbitrary and random manner.

If the yarn, whether in the close helix form of FIG. 4 or the open form of FIG. 5, is pulled out to its full length and released promptly, will return to its coiled form. If kept in an extended form under tension, it will gradually

assume a more extended form so that after a matter of say 30 minutes it will apparently lose all of its stretchiness. However, upon relaxation in an aqueous fluid, e.g., water or moist steam, it readily returns to the coiled form.

The last property can be taken advantage of in making fabrics from the novel yarn. Thus, referring to FIG. 2 of the drawing, plied yarn comprising cellulose fibers and 3 to 25% thermoplastic fibers are processed as described above and are then wrapped on a spool under tension. In accordance with normal procedures in the textile industry, considerable time elapses between the time when the yarn is spooled and the time when it is actually used on fabric making machinery, e.g., looms or knitting machines. In this time, the yarn, being under tension, has lost its stretchiness, so that it can be used on textile machinery as though it were conventional, non-stretch yarn. This is a very important practical advantage because the extreme extensibility of many stretch yarns makes them difficult to handle on conventional machinery. Once the fabric has been formed, it can be washed or steamed and the yarns tend to reacquire their shape prior to winding, imparting stretchability to the fabric itself.

As indicated in FIG. 3, it is also possible to make a stretch fabric by weaving or knitting plied yarns containing cellulosic filaments and 3 to 25% thermoplastic filaments, then treating the fabric with 5 to 40% caustic soda or its equivalent and finally heating to set the thermoplastic filaments. In such processes the details of concentration, time, temperature and the like are the same as discussed above in connection with the treatment of yarn as such.

The invention is illustrated by the following specific examples.

#### EXAMPLE I

A singles yarn comprising 10% Dacron (polyethylene terephthalate) staple and 90% of a high wet modulus<sup>1</sup> rayon staple, and having 30 turns per inch twist, in the Z direction, is plied to give a two ply yarn with 22 turns per inch twist in the S direction. The plied yarn is then wound into 110 meter skeins which are treated with an aqueous 16% NaOH at 20° C. for 1 minute. The skeins are then washed in water at 66° C. for 3 minutes, neutralized in 1% acetic acid for 3 minutes, again washed, extracted and dried at 121° C. for 5 minutes, followed by heating at 180° C. for 5 minutes. The resultant yarn has the appearance of FIG. 4.

The yarn is stretched to its maximum length, held for 10 seconds and then released. For maximum stretch,

$$\frac{\text{stretched length} - \text{original length}}{\text{original length}} \times 100$$

is 50%.

This is repeated ten times. The length of the yarn after final release is measured and the % growth is calculated as

$$\frac{\text{original length} - \text{final length}}{\text{original length}} \times 100$$

60 The recovery of the yarn is then calculated as

$$\frac{\text{percent stretch} - \text{percent growth}}{\text{percent stretch}} \times 100$$

65 and determined to be 50%.

#### EXAMPLE II

Yarn as made in Example I is reverse twisted 30 turns in the Z direction. A product having the appearance of the 70 yarn shown in FIG. 5 is obtained. When tested, as in Example I, it is found to have a maximum stretch of 160% and a recovery of 95%.

<sup>1</sup>The rayon has a dry tenacity of 5 grams per denier, a wet tenacity of 4 grams per denier and a stress of 2 grams per denier at 5% elongation when wet.

**5**  
**EXAMPLE III**

A plain weave fabric is made from the yarn described in Example I. The yarn is wound on spools, pulling out all stretch. Approximately 6 hours later yarn is drawn from the spools and fed to a single shuttle loom. After it is removed from the loom, the fabric is wet out with water at 80° C. for 10 minutes. It has a 200% stretch, and when held for 30 seconds and then released, has an 85% recovery. After being stretched for 40% and held for 5 minutes, it has a 95% recovery. This recovery increases upon standing, so that after 5 hours 99% recovery is obtained.

**EXAMPLE IV**

A plain weave fabric is made from the reverse twist yarn described in Example II. The yarn is wound on spools and in this operation all stretch is pulled out. Approximately 24 hours after winding, the yarn is woven, on a loom. After removal from the loom, the fabric is steamed, without tension, with saturated steam at atmospheric pressure. The fabric shrinks and becomes stretchy. It has a maximum stretch of 90%. Fabric samples are stretched 40%, held for various times and the percent recovery is recorded. Results are indicated below:

| Time Held Extended | Recovery percent   |                |                 |                 |
|--------------------|--------------------|----------------|-----------------|-----------------|
|                    | Imme-<br>di-<br>te | After<br>1 Hr. | After<br>3 Hrs. | After<br>5 Hrs. |
| 30 seconds         | 91                 | 98             | 98              | 98              |
| 5 minutes          | 90                 | 96             | 98              | 98              |

**EXAMPLE V**

A two-ply yarn, 10% Dacron and 90% high wet modulus rayon staple fiber is woven into a loose fabric. It is then treated, without tension, with an aqueous solution containing 16% NaOH at 20° C. for 3 minutes. After removal from the bath the fabric is neutralized, washed, dried and then heated at 176° C. for 2 minutes. A stretch fabric results.

**EXAMPLE VI**

Yarns made in accordance with Example II are knit into stockings on an 18-gauge circular knitting machine. After knitting, the stockings are placed in water at 66° C. for 5 minutes. After relaxation, one inch strips are cut from one of the stockings. Five inch reference marks are placed on one of the strips. It is then stretched along a calibrated scale to determine maximum stretch. A value of 200% is obtained.

**EXAMPLE VII**

The procedure of Example II is repeated with 3-ply yarns comprising singles yarns each containing 3% polypropylene staple fiber and 97% cotton fiber and twisted to 31 turns per inch in the Z direction. The plied yarn has 22 turns per inch in the S direction. The treating solution contains 25% NaOH. The yarn is heat treated at 150° C. for 180 seconds. In the reverse twist 32 turns per inch in the Z direction are inserted. The finished yarn has 190% maximum stretch and 82% recovery from maximum stretch after 10 seconds.

**EXAMPLE VIII**

A 24/2 yarn is spun from 90% conventional textile grade rayon staple fiber and 10% Dacron staple with 5.5 twist multiplier in the singles in the Z direction and with a ply twist of 22.5 turns per inch in the S direction. The yarn is treated in the skein without tension, in 25% aqueous NaOH at 20° C. for 2 minutes, rinsed in 65° C. water for 3 minutes, neutralized with 5% acetic acid,

rinsed with 20° C. water and dried relaxed. It is heated, relaxed, at 175° C. for 4 minutes and reverse twisted 31.8 turns per inch in the Z direction. The yarn has a maximum stretch of 206%, a recovery from maximum stretch after a 5 minute hold of 72% and a recovery after 25 maximum stretches, with immediate release, of 84%.

What is claimed is:

1. A method for making a stretch yarn which comprises treating a multi-ply yarn comprising between about 3% and about 25% by weight thermoplastic filaments and between about 75% and about 97% cellulose filaments, under substantially zero tension, with a swelling agent for cellulose equivalent to an aqueous solution containing between about 5% and about 40% NaOH and heating the treated yarn to set the thermoplastic filaments.
2. The method claimed in claim 1 and comprising twisting the yarn in a direction opposite to its ply beyond the point where there is no twist in the original plied yarn, after heat setting.
3. The method claimed in claim 1 wherein the cellulose filaments are selected from the group consisting of natural cellulose filaments and rayon filaments having a wet modulus of greater than about 1 gram per denier at 5% extension.
4. A method for making a stretch fabric which comprises treating a multi-ply yarn containing between about 3% and about 25% by weight thermoplastic filaments and the balance cellulose filaments, under substantially zero tension, with a swelling agent for cellulose equivalent to an aqueous solution containing 5 to 40% by weight NaOH, heating the treated yarn to set the thermoplastic filaments, subjecting the resulting yarn to tension until the stretch properties of the yarn are removed, converting the yarn to fabric and relaxing the fabric in an aqueous fluid to restore the stretch properties of the yarn.
5. The method claimed in claim 4 and comprising twisting the yarn in a direction opposite to its ply beyond the point where there is no twist in the original plied yarn, after heat setting.
6. The method claimed in claim 4 wherein the cellulose filaments are selected from the group consisting of natural cellulose filaments and rayon filaments having a wet modulus greater than about 1 gram per denier at 5% extension.
7. A method for making a stretch fabric which comprises converting a multi-ply yarn comprising cellulose filaments and between about 3 and about 25% by weight thermoplastic filaments, into a fabric, treating the fabric, in the substantial absence of tension, with a cellulose swelling agent equivalent in swelling power to an aqueous solution containing between about 5 and about 40% NaOH and then heat treating the fabric to set the thermoplastic filaments.
8. The method claimed in claim 7 wherein the cellulose filaments are selected from the group consisting of natural cellulose filaments and rayon filaments having a wet modulus greater than about 1 gram per denier at 5% extension.
9. A multi-ply stretch yarn produced according to the method of claim 1.
10. A stretch fabric produced according to the method of claim 4.
11. A stretch fabric produced according to the method of claim 7.

**References Cited**

**UNITED STATES PATENTS**

- |              |        |                        |           |
|--------------|--------|------------------------|-----------|
| 2,463,618    | 3/1949 | Heberlein et al. ----- | 57—157    |
| 70 2,919,534 | 1/1960 | Bolinger et al. -----  | 57—157 XR |
| 3,025,659    | 3/1962 | Stoddard et al. -----  | 28—72 XR  |

JOHN PETRAKES, Primary Examiner.